

# UNITED STATES PATENT OFFICE.

JAMES RAMSEY SPEER, OF TRAPPE, MARYLAND.

## CARBON-CHROME-NICKEL STEEL.

1,314,022.

Specification of Letters Patent. Patented Aug. 26, 1919.

No Drawing. Application filed June 15, 1918, Serial No. 240,211. Renewed April 26, 1919. Serial No. 292,982.

*To all whom it may concern:*

Be it known that I, JAMES RAMSEY SPEER, a resident of Trappe, in the county of Talbot and State of Maryland, have invented a new and useful Improvement in Carbon-Chrome-Nickel Steel, of which the following is a specification.

The present invention is an alloy steel, and particularly a hardened carbon-chrome-nickel steel, and the method of producing the same. The product comprises an alloy composed of relatively high carbon steel in combination with chromium and nickel, wherein the manganese, silicon, sulfur and phosphorus vary within the usual proportions for steel mixtures, and which product has the qualities hereinafter specified.

The object sought is a carbon-chrome nickel steel which is relatively simple to produce, at a comparatively low cost, which can be hardened and heat treated to a degree which classes it in performance with the most expensive and most difficult alloy mixtures known in the art, and which, when so hardened and heat treated, is very hard and tough and therefore well adapted to uses in which resistance to penetration from hard blows is a necessary quality.

Various special chrome-nickel steels have heretofore been made. Much has been written upon the subject and many patents for such alloy steels have been taken out. Practically all the literature, and the patents themselves, dwell upon the great difficulty of producing such alloys and place great emphasis upon the large amounts of nickel and chromium necessary to obtain the desired results. One conspicuous example of such prior nickel-chromium steel emphasizes the necessity of limiting the manganese content to less than .30%, also the exactness of the metallurgical operation in the production of the steel (practically to the destruction of the carbon, silicon and manganese content therein), and also the necessity of such exact metallurgical operation in order to produce the desired results. Prior investigators and inventors in this field have relied primarily upon the alloying elements, chromium and nickel, for the effects to be produced, and have added these elements, and especially the nickel, in large quantities.

According to my invention the carbon in the steel is primarily relied upon to produce the desirable qualities, and the alloying ele-

ments, chromium and nickel, are associated with it only in small amounts. In such association the chromium and nickel act merely to control and modify the form and characteristics of the carbon, and not directly because of their intrinsic qualities. The performance of my alloy depends primarily upon the various forms and character of the interlocking carbids, and because of the small quantities of chromium and nickel there is practically no risk of forming any of the oxides and ferro combinations which result from the use of large amounts of those elements. Because of the simplicity of this carbon control, the manufacture of the product is greatly simplified, and its cost of production is much reduced.

In steel alloys which are high in chromium and nickel, there is a certain lack of "digestion" of the chromium and nickel, and such alloys are subject to more than usual segregation. In the alloys which contain the higher percentages of chromium this is manifested by a great tendency to brittleness,—in some cases of almost explosive character. In the alloys which contain the higher percentages of nickel this is manifested by a lack of uniformity due to the segregation of the nickel which frequently gives serious trouble.

In my new alloy steel the relatively large quantity of carbon is merely controlled, and its effect strengthened, through and by means of the alloying compounds to "fix" the carbon in the best forms, as a result of which the product is capable of uses where the metal is subject to very severe service or abuse. Plates one-half inch thick made from my alloy, when properly quenched and heat treated, have resisted penetration of the latest United States Army model of armor-piercing bullet of 2800 feet muzzle velocity per second at a distance of fifty yards. This is the maximum test of resistance for such plates, thus showing that the alloy steel is admirably adapted for light armor such as is used for gun shields, armored tractors and automobiles, "tanks," and general ordnance work.

These one-half inch plates were rolled from a cast slab of initial thickness of 4 inches,—a reduction from 8 to 1,—which is one-fourth or even less of the reduction in rolling similar armor plates. Notwithstanding the limited working, this alloy steel

shows the best qualities of the most expensive steels, and its fineness of texture and silkiness of grain, together with its ability to respond to quenching and heat treatment, and its performance, make it particularly adapted for the uses already stated.

Brinnell hardness tests under different quenching and drawing treatments show that my alloy responds admirably to these treatments. The best results for light armor plates were shown when the plates were quenched from an initial temperature of  $1400^{\circ}$  to  $1450^{\circ}$  Fahrenheit. This quenching was limited to some extent, however, so that the plates were not cooled to too low a point from their initial heating. They were then reheated and drawn at a temperature of  $800^{\circ}$  to  $1000^{\circ}$  Fahrenheit, and then allowed to cool. These plates showed a Brinell hardness test of 370 to 418, and the best results for bullet resistance were obtained by drawing at  $850^{\circ}$  Fahrenheit, when the Brinell test showed about 418.

The relative degrees of hardness and toughness can be readily controlled by the heat treatment. For example, when the quenching was from the same initial temperature as that above given but was carried to a lower point and the plate again heated and drawn at a temperature of about  $600^{\circ}$  Fahrenheit and allowed to cool, the Brinnell hardness test showed about 500, but the plates were somewhat too brittle, and showed a tendency to crack under the bullet test named. On the other hand, when the quenching was from the same initial temperature, but not carried to so low a point, and the further heating and drawing was at a temperature close to  $1200^{\circ}$  Fahrenheit, the Brinnell test showed 250 to 300, and the plates were not quite so hard, but were very tough and resisted complete bullet penetration.

The analysis of the material in the above plates was as follows:

|            |       |
|------------|-------|
| Carbon     | 84 %  |
| Silicon    | .27 % |
| Manganese  | .59 % |
| Chromium   | .98 % |
| Nickel     | .60 % |
| Sulfur     | .022% |
| Phosphorus | .033% |

This alloy steel was made in an acid open hearth furnace, but could have been made in any suitable steel making furnace. It is not as high in carbon as some steels. The amount of chromium is just sufficient to "fix" the most resistant character or forms of the carbon combinations. The amount of nickel is just sufficient to counteract the tendency of the chromium and carbon combinations to produce brittleness, and to add some toughness to the matrix. The amount of manganese is just above the range of steels

of general character, but is much higher than that of special chrome-nickel steel alloys in which it has generally been considered necessary to keep the manganese low, that is, below .30% and preferably much lower. The chromium also is in excess of the nickel, thus reversing the usual, and long recognized as essential, relation between the chromium and nickel in such alloys. The proportions of silicon, sulfur and phosphorus in the above analysis correspond closely to such as are found in the better grade of steels. The qualities of the new alloy are due to the triple relation of the carbon modified by the chromium and both under the influence or effect of the nickel. The high carbon, controlled and modified as to its forms by the chromium and nickel, is primarily depended upon to produce the quality of hardness, and it is the determining factor in the excellence of the performance of the alloy and its susceptibility to ready control.

Various other analyses could be enumerated, but the one above given is sufficient to illustrate the principle of dependence on the carbon for the performance of the alloy; and yet its performance clearly takes it out of the class of high carbon steels. The proportion of carbon given, that is, .84%, is close to the middle of the carbon range, which may vary from .50% to 1.25%. The amount of carbon used depends upon the desired hardness of the alloy. The higher the carbon the greater is the degree of hardness obtained, and the lower the carbon the less the hardness of the alloy, with a relatively lower power of resistance. The amount of chromium and nickel to best modify and control the carbon and produce the interlocking functions and effects described may, and preferably will, be varied according to the amount of carbon present. The chromium may vary from .25% to 1.25%. The nickel may also vary from .25% to 1.25%, but generally will be present in a lesser amount than the chromium.

In producing the new alloy I follow the customary methods of steel makers, paying special attention, however, to the make-up of the raw materials in respect to their analyses, so that the figured analysis of the combination of the raw materials, after allowing for the losses incident to all steel making methods, will approach the analysis desired for the finished heat. In this manner and without other than ordinary skill on the part of the melter, the additions necessary to make the heats are reduced to a minimum, and the substantially complete destruction of the carbon, the silicon and the manganese (which some have heretofore thought necessary in the production of such alloy steel) is avoided, and this useless waste is turned to good account. In other words, I make use of the carbon, silicon and manga-

nese content of the raw materials charged into the furnace, and by reasonable care in refining in the furnace secure an analysis of the finished product within permissible variations from the analysis desired. Consequently, the method of producing the alloy is simple, is economical, and contrary to the heretofore suggested substantial destruction and elimination of such elements; and the 10 expensive ingredients, chromium and nickel, are added in quantities relatively low as compared with such elements in similar products as heretofore contemplated.

It is entirely feasible to add one or more 15 of the rarer alloying metals, to contribute somewhat to the variability of performance, but they are not essential.

I claim:

1. An alloy of steel characterized by great 20 hardness and toughness, variable by heat treatment, wherein steel of .50% to 1.25% carbon forms 97.50 to 99.50 parts, chromium

forms .25 to 1.25 parts, and nickel forms from .25 to 1.25 parts.

2. An alloy of steel characterized by great 25 hardness and toughness, variable by heat treatment, wherein steel of .50% to 1.25% carbon forms 97.50 to 99.50 parts, and chromium and nickel together form from .50 to 2.50 parts, the chromium being not less than 30 the nickel.

3. A hardened worked alloy of steel product characterized by great hardness and toughness, variable by heat treatment, wherein steel of .50% to 1.25% carbon forms 97.50 35 to 99.50 parts, and chromium and nickel together form from .50 to 2.50 parts, the chromium being not less than the nickel.

In testimony whereof I have hereunto set my hand.

JAMES RAMSEY SPEER.

Witness:

HARVEY T. WINFIELD.